# EUROPEAN PATENT SPECIFICATION

(11) **EP 4 590 894 B1**
(45) Date of publication and mention of the grant of the patent: **05.11.2025**
(21) Application number: 23836479.8
(22) Date of filing: 20.12.2023
(51) Int. Cl.: D21C 1/02, D21B 1/02, D21B 1/30, D21C 1/06, D21C 3/02, D21H 11/02

(54) **PRODUCTION OF CTMP FROM A HARDWOOD/SOFTWOOD MIXTURE**
HERSTELLUNG VON CTMP AUS EINER HARTHOLZ/WEICHHOLZ-MISCHUNG
PRODUCTION DE CTMP À PARTIR D'UN MÉLANGE DE BOIS DUR/BOIS MOU

(30) Priority: 21.12.2022 EP 22215622
(43) Date of publication of application: 30.07.2025
(73) Proprietor: Billerud Aktiebolag (publ), 169 27 Solna (SE)
(72) Inventor: LINDSTEDT, Thomas, 653 45 Karlstad (SE); GRANFELDT, Thomas, 865 33 Alnö (SE); ENGSTRAND, Per, 616 33 Åby (SE)
(74) Representative: Kransell & Wennborg KB
(86) International application number: PCT/EP2023/086959
(87) International publication number: WO 2024/133460

(56) References cited:
- US-A- 4 486 267
- US-A- 4 798 651

## Description

### TECHNICAL FIELD

The present invention relates to the field of chemithermomechanical pulp (CTMP) and in particular the production thereof.

### BACKGROUND

Chemithermomechancial pulp (CTMP) is a high yield pulp which can provide a high bulk and has been used since 1960s. CTMP is produced by mild chemical impregnation of wood chips, followed by a heat treatment to soften the wood. The treated wood chips are then subjected to defibration/refining (typically in several steps) and optionally bleaching. The obtained CTMP typically has comparatively high bulk, preferably in combination with low shives content. The process can be further improved by using higher temperatures during the heat treatment. Using steam of relatively high temperature in the heat treatment typically leads to a decrease in the energy input needed during the pressurized defibration step.

Document US4486267A discloses a process for producing hardwood chemithermomechanical pulp, comprising a two-step impregnation of hardwood chips containing 60% maple.

### SUMMARY

It is an objective of the present disclosure to enable production of a chemithermomechanical pulp (CTMP) of improved properties.

Accordingly, there is provided a method of forming a high temperature chemithermomechanical pulp (HT-CTMP) comprising the steps of:
a) mixing hardwood chips and softwood chips to obtain a mixture, wherein the dry weight ratio of hardwood to softwood in said mixture is between 85:15 and 65:35;
b) impregnating the chips of the mixture with an impregnation liquid comprising sulfite and optionally NaOH to obtain impregnated chips;
c) applying steam having a temperature of at least 150°C to the impregnated chips to obtain pretreated chips; and
d) defibrating the pretreated chips,
wherein the mass flow of sulfite (calculated as Na₂SO₃) to step b) is higher than the mass flow of NaOH to step b) and the residence time in step c) is no more than two minutes.

### BRIEF DESCRIPTION OF THE DRAWINGS

Figures 1-3 show exemplary embodiments of a full-scale system for producing HT-CTMP according to the present disclosure.
Figure 4 show results obtained in the pilot trial described below.

### DETAILED DESCRIPTION

There is provided a method of forming a high temperature chemithermomechanical pulp (HT-CTMP) comprising the steps of:
a) mixing hardwood chips and softwood chips to obtain a mixture, wherein the dry weight ratio of hardwood to softwood in said mixture is between 85:15 and 65:35;
b) impregnating the chips of the mixture with an impregnation liquid comprising sulfite and optionally NaOH to obtain impregnated chips;
c) applying steam having a temperature of at least 150°C to the impregnated chips to obtain pretreated chips; and
d) defibrating the pretreated chips,
wherein the mass flow of sulfite (calculated as Na₂SO₃) to step b) is higher than the mass flow of NaOH to step b) and the residence time in step c) is no more than two minutes.

The chips from step a) are typically washed and then pre-steamed before being impregnated in step b). Embodiments of the washing and pre-steaming as well as other preparatory steps are described in the examples section below.

The mass flow of sulfite (calculated as Na₂SO₃) to step b) is preferably at least 50% higher than the mass flow of NaOH to step b). In one embodiment, the mass flow of sulfite (calculated as Na₂SO₃) to step b) is at least 100% higher than the mass flow of NaOH to step b).

The present inventors have realized that a HT-CTMP of satisfactory properties can be produced without supplying any NaOH or other alkali to step b). Alternatively, NaOH may be supplied to step b), but in an amount not greater than 15 kg/tonne dry wood chips, such as not greater than 10 kg/tonne dry wood chips. A low amount of NaOH or no NaOH may be associated with an increased tensile index of the HT-CTMP. Furthermore, using a low amount of NaOH may result in an increase in bulk.

The mass flow of sulfite (calculated as Na₂SO₃) to step b) may be 5-30 kg per tonne dry wood chips, such as 10-30 kg per tonne dry wood chips, such as 10-28 kg per tonne dry wood chips, such as 15-28 kg per tonne dry wood chips, such as 5-20 kg per tonne dry wood chips, such as 5-15 kg per tonne dry wood chips. The addition of sulfite in the impregnation liquid may increase the brightness of the HT-CTMP prior to bleaching and thus a pulp with a higher bulk can be obtained at a given brightness after bleaching.

The pH of the impregnation liquid is below 10.9. Such a pH reflects that no or only a small amount of NaOH has been added to the sulfite-containing impregnation liquid.

The hardwood chips may be birch wood chips or maple wood chips. The softwood chips may be spruce wood chips.

In one embodiment, the steam temperature in step c) is at least 155°C, such as at least 160°C. An upper limit for the steam temperature in step c) may be 190°C.

In one embodiment, the steam temperature in step c) is at least 160°C, the alkali supply in step b) is less than 10 kg/tonne dry wood chips and the impregnated chips are defibrated to a CSF of 700 ml or more. This promotes high bulk in the HT-CTMP.

The dry weight ratio of hardwood to softwood in said mixture is preferably between 80:20 and 65:35, such as between 72:25 and 65:35.

The temperature of the impregnation liquid is preferably at least 70°C, such as 70°C-99°C, such as 80°C-99°C. At such a relatively high temperature, the viscosity of the impregnation liquid is lower, which facilitates the absorption thereof.

In step b), the chips may be fed to an impregnation zone comprising the impregnation liquid using a plug screw (or another compressing device) such that the chips expand in the impregnation zone and absorb the impregnation liquid, thereby providing the impregnated chips.

In another embodiment, step b) comprises:
- feeding the chips to a pre-impregnation zone comprising a pre-impregnation liquid using a plug screw (or another compressing device) such that the pre-steamed chips expand in the pre-impregnation zone and absorb the pre-impregnation liquid, thereby providing pre-impregnated chips; and
- feeding the pre-impregnated chips to an impregnation zone comprising an impregnation liquid using a plug screw (or another compressing device) such that the pre-impregnated chips expand in the impregnation zone and absorb the impregnation liquid, thereby providing the impregnated chips.

In this embodiment, the temperatures of the pre-impregnation liquid and the impregnation liquid are preferably at least 70°C, such as 70°C-99°C, such as 80°C-99°C. At such temperatures, the viscosity of the liquids is lower, which facilitates the absorption thereof.

In one embodiment, the impregnated chips obtained in step b) are transferred to step c) without compressing the impregnated chips. Hence, no plug screw is used for the transfer of the impregnated chips in this embodiment. Instead, the transfer of the impregnated chips may comprise lifting the impregnated chips out of the impregnation liquid using a transport screw and then allowing the impregnated chips to fall into a heating zone in which the steam-based heat-treatment of step c) takes place.

The defibration of step d) is typically carried out under pressure.

The pulp obtained from step d) may be subjected to refining (such as low consistency refining) and/or bleaching. Embodiments of such refining and/or bleaching are described in the examples section below with reference to figures 1-3.

### EXAMPLES

### Pilot trial 1

Two batches of wood chips were prepared:
Batch 1 - 100 dry wt.% birch wood chips; and
Batch 2 - 70 dry wt.% birch wood chips and 30 dry wt.% spruce chips

After washing, the chips of each batch were subjected to pre-steaming for 10 minutes using atmospheric steam.

The chips were then impregnated with an aqueous impregnation liquid comprising NaOH, Na₂SO₃ and DTPA in an impregnation vessel of a pilot plant. The washed and pre-steamed chips were fed to the impregnation vessel using a plug screw such that the chips expanded in the impregnation liquid, which had a temperature of 40°C.

NaOH, Na₂SO₃ and DTPA were supplied to the impregnation vessel in amounts of 10, 20 and 2 kg per tonne dry chips, respectively.

The impregnated chips were then heated by the application of steam having a temperature of 165°C. No plug screw was used to transfer the chips from the impregnation to the steaming step. Hence, the chips were transferred to the steaming step without being compressed. The residence time in the steaming step was less than two minutes. The pretreated chips from the steaming step were subjected to different degrees of high consistency defibration such that pulps were obtained. Properties of the pulps were then measured (see table 1 below). Further, sheets were formed from the pulps according to ISO 5269-1 and properties of the sheets were measured.

**Table 1. Pulp and sheet properties. "Deg. of HC defib." means degree of high consistency defibration and is the specific energy consumption (kWh/dry tonne wood chips) in the defibration step.**

| Batch | Birch/Spruce (wt.%/wt.%) | Deg. of HC defib. | CSF (ml) | Shives (%) | Bulk (cm³/g) | Tensile index (Nm/g) |
|---|---|---|---|---|---|---|
| 1 | 100/0 | 615 | 719 | 0.17 | 5.03 | 3.3 |
| 1 | 100/0 | 1103 | 610 | 0.10 | 4.17 | 7.5 |
| 2 | 70/30 | 540 | 715 | 0.43 | 5.13 | 6.8 |
| 2 | 70/30 | 852 | 614 | 0.09 | 4.14 | 13.1 |

As shown in table 1, the 70/30 mixture (batch 2) resulted in considerably higher tensile index values than 100% birch (batch 1) at comparable freeness, shives and bulk values. The relationship between bulk and tensile index is also illustrated in figure 4, which shows significantly tensile index (i.e. strength) at a given bulk for batch 2.

### Pilot trial 2

A pilot trial was performed using maple wood chips (average length = 18 mm) and spruce wood chips (average length = 18 mm). Before being used in the pilot trial, the maple wood chips were soaked in water overnight.

Subsequently, three batches of wood chips were prepared:
Batch 3 - 100 dry wt.% maple wood chips;
Batch 4 - 85 dry wt.% maple wood chips and 15 dry wt.% spruce wood chips; and
Batch 5 - 70 dry wt.% maple wood chips and 30 dry wt.% spruce wood chips.

After washing, the chips of each batch were subjected to pre-steaming for 10 minutes using atmospheric steam.

The chips were then impregnated with an aqueous impregnation liquid comprising NaOH, Na₂SO₃ and DTPA in an impregnation vessel of a pilot plant. The washed and pre-steamed chips were fed to the impregnation vessel using a plug screw such that the chips expanded in the impregnation liquid, which had a temperature of 40°C.

Na₂SO₃ and DTPA were supplied to the impregnation vessel in amounts of 20 and 2 kg per tonne dry chips, respectively. The amount of NaOH supplied varied from 0-10 kg per tonne dry chips, see table 2.

The impregnated chips were then heated by the application of steam having a temperature of 165 °C. No plug screw was used to transfer the chips from the impregnation to the steaming step. Hence, the chips were transferred to the steaming step without being compressed. The residence time in the steaming step was less than two minutes. The pretreated chips from the steaming step were subjected to different degrees of high consistency defibration such that pulps were obtained. Properties of the pulps were then measured, see table 2. Further, sheets were formed from the pulps according to ISO 5269-1 and properties of the sheets were measured.

**Table 2. Pulp and sheet properties. "Deg. of HC defib." means degree of high consistency defibration and is the specific energy consumption (kWh/dry tonne wood chips) in the defibration step.**

| Batch | Maple/Spruce (wt.%/wt.%) | NaOH (kg) | Deg. of HC defib. | CSF (ml) | Shives (%) | Bulk (cm³/g) | Tensile index (Nm/g) |
|---|---|---|---|---|---|---|---|
| 3 | 100/0 | 9 | 620 | 659 | 0.32 | 4.41 | 3.3 |
| 4 | 85/15 | 10 | 735 | 598 | 0.29 | 4.34 | 6.4 |
| 5 | 70/30 | 10 | 737 | 636 | 0.38 | 4.19 | 7.4 |
| 5 | 70/30 | 0 | 916 | 595 | 0.24 | 4.38 | 8.4 |

As shown in table 2, the 85/15 mixture (batch 4) and 70/30 mixture (batch 5) resulted in considerably higher tensile index values than 100% maple (batch 3) at comparable freeness, shives and bulk values. Furthermore, a reduction in the amount of NaOH in the impregnation liquid from 10 kg/tonne to 0 kg/tonne further increased the tensile index and bulk.

### Exemplary embodiment of a full-scale system for producing HT-CTMP

Figures 1-3 illustrate exemplary embodiments of a full-scale system for producing HT-CTMP.

A chipper 101 is used to prepare chips from hardwood (e.g. birch wood) and softwood (e.g. spruce wood). It may be preferred to prepare hardwood chips that are relatively short, such as < 20 mm, to aid impregnation. Spruce wood chips are generally easier to impregnate and can hence be longer, such as 22-24 mm. However, the spruce chips may also have the same length as the hardwood chips. The settings of a conventional wood chipper can be adjusted to achieve desired chip lengths. Shorter chips from such a chipper are also thinner.

The hardwood chips and the spruce wood chips from the chipper 101 are stored in a hardwood chips silo 102a and a softwood chips silo 102b, respectively. A chips mixing system 103 is arranged downstream the silos 102a, 102b to prepare a chips mixture having the desired ratio of hardwood chips to spruce wood chips. This ratio is in the range of 85:15 to 65:35 (based on dry weight).

The chips from the chips mixing system 103 are optionally stored in an aerobic environment in a maturation silo 104 for a period of at least 24 h (typically about 72 h). A typical temperature in the maturation silo 104 is 60°C, which can be achieved by feeding low-pressure steam into the maturation silo 104. The treatment of the chips in the maturation silo 104 degrades triglycerides. The degradation products can then be extracted in downstream process steps.

Another option is to design the chip silos 102a, 102b as maturation silos. A benefit of this option is that the maturation time and temperature can be individually adapted to the respective wood types.

Yet another option is to place the maturation silo 104 between the chips washing arrangement 106 and the pre-steaming bin 107 described below. It is also possible to omit the maturation step.

Before being impregnated, the chips are washed in a chips washing arrangement 106. Upstream the chips washing arrangement 106, a conditioning device 105 may be arranged. The conditioning device 105 is typically a chip steaming bin. The purpose of the conditioning device 105 is to provide chips of fairly constant temperature. The conditioning device 105 may also, to some extent, reduce variations in moisture content. During cold winter months, ice on the chips is melted in the conditioning device 105, which facilitates the downstream washing and processing. Hence, the conditioning device 105 may be particularly advantageous when there is no upstream maturation silo. In case there is an upstream maturation silo, the conditioning device 105 may be omitted.

In the chips washing arrangement 106, the chips are typically soaked and agitated in water and then dewatered. The washed and dewatered chips are then steamed in a pre-steaming bin 107. The residence time of the chips in the pre-steaming bin 107 is typically at least 10 min.

The steamed chips from the pre-steaming bin 107 are subjected to impregnation in one or two steps.

In case of one-step impregnation, a plug screw 108 feeds the steamed chips into a reactor 109. The steamed chips, which were compressed in the plug screw 108, expands in a bath of aqueous impregnation liquid 110 in the reactor 109. During the expansion, the chips absorb impregnation liquid. The temperature of the impregnation liquid is preferably 80°C-99°C. The impregnation liquid, which is aqueous, comprises sulfite (added as Na₂SO₃) and optionally alkali (e.g. NaOH). If included, the concentration of NaOH in the impregnation liquid is lower than that of Na₂SO₃. The (expanded and impregnated) chips are lifted from the bath of impregnation liquid 110 by means of a transport screw 111 and are then allowed to fall over an edge 112 and into steaming area 113 of the reactor 109, in which they are heated by steam having a temperature of at least 150°C. The chips treated in the reactor 109 are transferred to a chips defibrator 114 without flashing off any steam on the way. The residence time in the steaming area 113 is less than two minutes.

In case of two-step impregnation, a plug screw 115 feeds the steamed chips into a pre-impregnation chamber 116. The steamed chips, which were compressed in the plug screw 115, expands in a bath of pre-impregnation liquid 117 in the pre-impregnation chamber 116. During the expansion, the chips absorb pre-impregnation liquid. The temperature of the pre-impregnation liquid is preferably 80°C-99°C. The pre-impregnation liquid is water that may comprise alkali and optionally sulfite. The (expanded and impregnated) chips are lifted from the bath of pre-impregnation liquid 117 by means of a transport screw 118. A plug screw 119 then feeds the pre-impregnated chips into a reactor 120. The pre-impregnated chips, which were compressed in the plug screw 119, expands in a bath of impregnation liquid 121 in the reactor 120. During the expansion, the chips absorb impregnation liquid, which preferably has a temperature of 80°C-99°C. The impregnation liquid, which is aqueous, comprises sulfite and optionally some alkali. The (expanded and impregnated) chips are lifted from the bath of impregnation liquid 121 by means of a transport screw 122 and are then allowed to fall over an edge 123 and into steaming area 124 of the reactor 120, in which they are heated by steam having a temperature or at least 150°C (as a consequence of the steam temperature, the final product is a HT-CTMP). The residence time in the steaming area 124 is less than two minutes. The chips treated in the reactor 120 are transferred to the chips defibrator 114 without flashing off any steam on the way.

In the chips defibrator 114, the dry matter content may be about 45%-50% (in case there is no plug screw between the steaming area 124 and the chips defibrator 114, the dry matter content may however be as low as 30%). The pulp from the chips defibrator 114 is subjected to flashing in a steam separator 125 and then pulped in a first pulper 126. The pulp from the first pulper 126 is then treated in a first dewatering press 127. The pressate from the first dewatering press 127 contains extractives (and dissolved wood substances and residual chemicals) that are unwanted in the final CTMP product. Separation of extractives by pressing in this position is advantageous since the pulp still has very high freeness (typically >650 ml or even >700 ml) and is thus easily dewatered. Limiting the residence time in the first pulper 126 to below 10 min (typically about 3 min) is advantageous since it limits the time available to the extractives to be adsorbed onto the fibers before the first dewatering press 127.

The pulp from the first dewatering press 127 has undergone chemical treatment, heat treatment by high temperature steam and mechanical treatment (i.e. defibration) and it thus a HT-CTMP. This pulp may be used in the production of paperboard without further chemical treatment or refining. I may also be subjected to low consistency (LC) refining before being used in paperboard production. Yet another option is to further treat the pulp by bleaching and LC refining as described below.

The pulp from the first dewatering press 127 is subjected to middle consistency (MC) bleaching in a MC bleach tower 128 using unreacted peroxide from the downstream high consistency (HC) bleaching and, if needed, make-up quantities of NaOH and peroxide. MC means 10%-12%. The MC-bleached pulp is treated in a second dewatering press 129 also producing a pressate. The pulp from the second dewatering press 129 is subjected to high consistency (HC) bleaching in a HC bleach tower 130 using fresh peroxide and alkali (and optionally a peroxide stabilizer, such as a silicate or a non-silicate stabilizer and/or a chelating agent, such as DTPA or EDTA). The HC-bleached pulp from the HC bleach tower 130 are pulped in a second pulper 131 (residence time: <10 min, such as about 3 min) to produce a pulp having a consistency of about 4%-6%. This pulp is then subjected to low consistency (LC) refining in LC refiners 132. A third dewatering press 133 then separates a third pressate from the LC-refined pulp. The fibers from the third dewatering press 133 are pulped in a third pulper 134 (residence time: <10 min, such as about 3 min) to produce a pulp having a consistency of 2%-4%. Screens 135 are then used to separate a reject from the pulp from the third pulper 134. The separated reject is collected in a reject tank 136.

The design of the remaining parts of the system depends on if only market pulp is produced (i.e. all CTMP is subjected to flash drying and baling) or if there is an adjacent board-making machine to which at least part of the CTMP is supplied without drying.

In the former case, which is illustrated in figure 2, the pulp from the screens 135 are cleaned in cleaners 137 to provide cleaned pulp and second reject that is collected in a second reject tank 138. The cleaned pulp is then filtered in a disc filter 139 and collected in a MC tower 140. From the pulp from the MC tower 140, a fourth dewatering press 141 produces dewatered fibers and a fourth pressate. The dewatered fibers are led to an arrangement for fiber treatment and shredding 142 and then to a flash drying arrangement 143. Finally, bales of the dried fibers from the flash drying arrangement 143 are formed in a baling arrangement 144.

In the latter case, which is illustrated in figure 3, the pulp from the screens is filtered in a disc filter 145 and treated in a fourth dewatering press 146 such that a fourth pressate and an MC pulp are obtained. The MC pulp is collected in a MC tower 147.

To produce (dried) market pulp, a fifth dewatering press 148 produces dewatered fibers and a fifth pressate from MC pulp from the MC tower 147. The dewatered fibers are led to an arrangement for fiber treatment and shredding 149 and then to a flash drying arrangement 150. Finally, bales of the dried fibers from the flash drying arrangement 150 are formed in a baling arrangement 151.

To use the produced CTMP in the production of paperboard, MC pulp from the MC tower 147 is led to a board-making machine.

## Claims

1. A method of forming a high temperature chemithermomechanical pulp (HT-CTMP) comprising the steps of:
a) mixing hardwood chips and softwood chips to obtain a mixture, wherein the dry weight ratio of hardwood to softwood in said mixture is between 85:15 and 65:35;
b) impregnating the chips of the mixture with an impregnation liquid comprising sulfite and optionally NaOH to obtain impregnated chips;
c) applying steam having a temperature of at least 150°C to the impregnated chips to obtain pretreated chips; and
d) defibrating the pretreated chips,
wherein the mass flow of sulfite (calculated as Na₂SO₃) to step b) is higher than the mass flow of NaOH to step b) and the residence time in step c) is no more than two minutes.

2. The method of claim 1, wherein the mass flow of sulfite (calculated as Na₂SO₃) to step b) is at least 50% higher than the mass flow of NaOH to step b).

3. The method of claim 1, wherein the mass flow of sulfite (calculated as Na₂SO₃) to step b) is at least 100% higher than the mass flow of NaOH to step b).

4. The method of claim 1, wherein no NaOH or other alkali is supplied to step b).

5. The method of any one of the preceding claims, wherein the pH of the impregnation liquid is below 10.9.

6. The method of any one of the preceding claims, wherein the hardwood chips are birch wood chips.

7. The method of any one of the preceding claims, wherein the softwood chips are spruce wood chips.

8. The method of any one of the preceding claims, wherein the steam temperature in step c) is at least 155°C, such as at least 160°C.

9. The method of any one of the preceding claims, wherein the mass flow of sulfite (calculated as Na₂SO₃) to step b) is 5-30 kg per tonne dry wood chips, such as 10-30 kg per tonne dry wood chips, such as 15-25 kg per tonne dry wood chips.

10. The method of any one of the preceding claims, wherein the dry weight ratio of hardwood to softwood in said mixture is between 80:20 and 65:35, such as between 72:25 and 65:35.

11. The method of any one of preceding claims, wherein the impregnated chips obtained in step b) are transferred to step c) without compressing the impregnated chips.

12. The method of any one of preceding claims, wherein step b) comprises feeding the chips to an impregnation zone comprising the impregnation liquid using a plug screw such that the chips expand in the impregnation zone and absorb the impregnation liquid, thereby providing the impregnated chips.

## Patentansprüche

1. Verfahren zum Herstellen eines hochtemperaturchemothermomechanischen Zellstoffs (HT-CTMP), umfassend die Schritte:
a) Mischen von Hartholz- und Weichholzspänen, um ein Gemisch zu erhalten, wobei das Trockengewichtsverhältnis von Hartholz zu Weichholz in dem Gemisch zwischen 85:15 und 65:35 liegt;
b) Imprägnieren der Späne des Gemischs mit einer Imprägnierflüssigkeit, die Sulfit und optional NaOH umfasst, um imprägnierte Späne zu erhalten;
c) Beaufschlagen der imprägnierten Späne mit Dampf mit einer Temperatur von mindestens 150 °C, um vorbehandelte Späne zu erhalten; und
d) Defibrillieren der vorbehandelten Späne,
wobei der Massenstrom an Sulfit (berechnet als Na₂SO₃), der in Schritt b) zugeführt wird, größer ist als der Massenstrom an NaOH, der in Schritt b) zugeführt wird, und die Verweilzeit in Schritt c) höchstens zwei Minuten beträgt.

2. Verfahren nach Anspruch 1, wobei der Massenstrom an Sulfit (berechnet als Na₂SO₃), der in Schritt b) zugeführt wird, mindestens 50 % höher ist als der Massenstrom an NaOH, der in Schritt b) zugeführt wird.

3. Verfahren nach Anspruch 1, wobei der Massenstrom an Sulfit (berechnet als Na₂SO₃), der in Schritt b) zugeführt wird, mindestens 100 % höher ist als der Massenstrom an NaOH, der in Schritt b) zugeführt wird.

4. Verfahren nach Anspruch 1, wobei in Schritt b) kein NaOH oder ein anderes Alkali zugeführt wird.

5. Verfahren nach einem der vorhergehenden Ansprüche, wobei der pH-Wert der Imprägnierflüssigkeit unter 10,9 liegt.

6. Verfahren nach einem der vorhergehenden Ansprüche, wobei die Hartholzspäne Birkenspäne sind.

7. Verfahren nach einem der vorhergehenden Ansprüche, wobei die Weichholzspäne Fichtenspäne sind.

8. Verfahren nach einem der vorhergehenden Ansprüche, wobei die Dampftemperatur in Schritt c) mindestens 155 °C, beispielsweise mindestens 161 °C, beträgt.

9. Verfahren nach einem der vorhergehenden Ansprüche, wobei der Massenstrom an Sulfit (berechnet als Na₂SO₃), der in Schritt b) zugeführt wird, 5-30 kg pro Tonne trockene Holzspäne beträgt, beispielsweise 10-30 kg pro Tonne trockene Holzspäne, beispielsweise 15-25 kg pro Tonne trockene Holzspäne.

10. Verfahren nach einem der vorhergehenden Ansprüche, wobei das Trockengewichtsverhältnis von Hartholz zu Weichholz in dem Gemisch zwischen 80:20 und 65:35, beispielsweise zwischen 72:25 und 65:35, liegt.

11. Verfahren nach einem der vorhergehenden Ansprüche, wobei die in Schritt b) erhaltenen imprägnierten Späne in Schritt c) ohne Verdichtung überführt werden.

12. Verfahren nach einem der vorhergehenden Ansprüche, wobei Schritt b) das Zuführen der Späne zu einer Imprägnierzone mit der Imprägnierflüssigkeit unter Verwendung einer Stopfschnecke umfasst, so dass sich die Späne in der Imprägnierzone ausdehnen und die Imprägnierflüssigkeit aufnehmen, wodurch die imprägnierten Späne bereitgestellt werden.

## Revendications

1. Procédé de formation d'une pâte chimico-thermo-mécanique à haute température (CTMHT) comprenant les étapes suivantes :
a) le mélange de copeaux de bois dur et de copeaux de bois tendre pour obtenir un mélange, dans lequel le rapport en poids sec du bois dur au bois tendre dans ledit mélange est compris entre 85:15 et 65:35 ;
b) l'imprégnation des copeaux du mélange avec un liquide d'imprégnation comprenant du sulfite et éventuellement du NaOH pour obtenir des copeaux imprégnés ;
c) l'application de vapeur à une température d'au moins 150 °C aux copeaux imprégnés pour obtenir des copeaux prétraités ; et
d) le défibrage des copeaux prétraités,
dans lequel le débit massique de sulfite (calculé en termes de Na₂SO₃) à l'étape b) est supérieur au débit massique de NaOH à l'étape b) et le temps de séjour à l'étape c) n'est pas supérieur à deux minutes.

2. Procédé selon la revendication 1, dans lequel le débit massique de sulfite (calculé en termes de Na₂SO₃) vers l'étape b) est au moins 50 % supérieur au débit massique de NaOH vers l'étape b).

3. Procédé selon la revendication 1, dans lequel le débit massique de sulfite (calculé en termes de Na₂SO₃) vers l'étape b) est au moins 100 % supérieur au débit massique de NaOH vers l'étape b).

4. Procédé selon la revendication 1, dans lequel aucun NaOH ou autre alcali n'est fourni à l'étape b).

5. Procédé selon l'une quelconque des revendications précédentes, dans lequel le pH du liquide d'imprégnation est inférieur à 10,9.

6. Procédé selon l'une quelconque des revendications précédentes, dans lequel les copeaux de bois dur sont des copeaux de bois de bouleau.

7. Procédé selon l'une quelconque des revendications précédentes, dans lequel les copeaux de bois tendre sont des copeaux de bois d'épicéa.

8. Procédé selon l'une quelconque des revendications précédentes, dans lequel la température de la vapeur à l'étape c) est d'au moins 155 °C, telle qu'au moins 160 °C.

9. Procédé selon l'une quelconque des revendications précédentes, dans lequel le débit massique de sulfite (calculé en termes de Na₂SO₃) vers l'étape b) est compris entre 5 et 30 kg par tonne de copeaux de bois secs, tel que compris entre 10 et 30 kg par tonne de copeaux de bois secs, tel que compris entre 15 et 25 kg par tonne de copeaux de bois secs.

10. Procédé selon l'une quelconque des revendications précédentes, dans lequel le rapport en poids sec entre le bois dur et le bois tendre dans ledit mélange est compris entre 80:20 et 65:35, tel que compris entre 72:25 et 65:35.

11. Procédé selon l'une quelconque des revendications précédentes, dans lequel les copeaux imprégnés obtenus à l'étape b) sont transférés à l'étape c) sans compression des copeaux imprégnés.

12. Procédé selon l'une quelconque des revendications précédentes, dans lequel l'étape b) comprend l'alimentation des copeaux vers une zone d'imprégnation comprenant le liquide d'imprégnation à l'aide d'une vis sans fin de manière à ce que les copeaux se dilatent dans la zone d'imprégnation et absorbent le liquide d'imprégnation, fournissant ainsi les copeaux imprégnés.
